

Sept. 21, 1965

R. J. MILLER

3,207,073

## EXPLOSIVE CORD AND ASSEMBLY

Filed Dec. 21, 1962

**FIG. I**



**FIG. 2**

FIG. 3



**FIG. 4**

FIG. 5



INVENTOR  
ROSS JAY MILLER

BY John H. Tregoning  
ATTORNEY

1

3,207,073

**EXPLOSIVE CORD AND ASSEMBLY**

Ross Jay Miller, Franklin Lakes, N.J., assignor to E. I. du Pont de Nemours and Company, Wilmington, Del., a corporation of Delaware

Filed Dec. 21, 1962, Ser. No. 246,537

7 Claims. (Cl. 102—27)

This application is a continuation-in-part of U. S. patent application Serial No. 33,716, filed June 3, 1960, now abandoned.

The present invention relates to a novel delay-initiation cord for use in delay blasting and to a novel blasting assembly.

It has been generally recognized in blasting practice that improved results are obtained when the charges in all the boreholes for the blast are not initiated simultaneously, but are initiated in sequence and at precise intervals of time. Such non-simultaneous initiation, usually referred to as delay blasting, provides greater and more efficient blasting action, i.e., both the amount of material, or burden, blasted in one operation and the degree of fragmentation are substantially improved. This substantial improvement over the instantaneous method of initiation is due primarily to the fact that the burden loosened by the initial charge has moved out from the face a distance before the next charge is initiated. Thus, in effect, a "peeling-off" action is obtained. Greatly lessened ground vibration is another desirable feature of delay blasting. A further advantage is that owing to the greater burden movement, the cost of drilling and of explosives are reduced considerably.

Several means have been employed to accomplish the desired delayed initiation of the explosive charges. One means involves a mechanical arrangement for controlling the application of electrical energy to the individual electric initiators. Another means is a delay electric initiator in which the delay interval is provided by the burning of a pyrotechnic composition (a delay charge) interposed between the electrically ignited charge and the primer charge of the initiator. A third means is the positioning of a delay connector in a line of detonating fuse ("Primacord") leading to the explosive charge. A fourth means involves the low-energy connecting cord as described in U. S. 2,982,210, which transmits a detonation impulse to a delay connector or to a delay initiator.

All of the foregoing procedures suffer from certain serious shortcomings. The electrically initiated devices possess the disadvantage of being subject to accidental firing by stray currents, lightning, or radio frequency energy. Further, the delay intervals provided by the electric initiators now commercially available are not always as accurate as might be desirable. Delay blasting with detonating fuse and delay connectors, while free of the hazards associated with electrical firing means, is, nevertheless, far from an ideal method. One particularly disturbing aspect of this method is the considerable noise and brisance produced by the fuse upon detonation. Aside from the annoyance to individuals in the vicinity which this noise creates, the attendant brisance also necessitates careful positioning of the fuse, often with elaborate and expensive shielding methods, to prevent "cut-offs" or severing of the fuse.

Further, the delay connectors, in every case of which I am aware comprise units which are manufactured in a few standard sizes and impose upon the blaster a limited scope of operation. Moreover, owing to their tendency to fail in operation, such devices commonly are employed in parallel in an assembly generally in a secondary or supplementary trunk line of detonating fuse in the hope if one assembly of cord and connectors does not function properly, the other probably will. Further, many of the

2

connectors and delay assemblies presently available are of the one-way type and necessitate a precise order of rotation. The low-energy connecting cord, while free of objectionable brisance, necessitates careful handling of the cord and connectors or initiators so that the two will not become separated. Additionally, the low-energy assemblies also are manufactured in a few standard sizes which limit the scope of blasting operation. All of the aforementioned methods of producing a delayed blast require expensive and elaborate accessories and great caution and careful supervision in loading the explosive charges and in making the necessary and tedious connections for the blast.

A most serious shortcoming of delay blasting means used heretofore, each of which relies upon delay connectors and/or delay detonators, is that despite every manufacturing precaution, delay periods of supposedly equal connectors or detonators are not only unequal, but frequently may vary appreciably from the desired time. Thus, while the average delay time for any large sampling may be close to the design interval, many individual units may have delay times appreciably greater or less than the design interval. Consequently, the danger exists that a detonator or connector having the maximum delay time of one delay series may have the same or even a longer delay time than that having the minimum delay time in the next one or several delay series. If such detonators or connectors are used together in the field, obviously the desired blasting cannot be achieved, in fact harmful action may occur.

In accordance with this invention, a means for delay blasting is provided in which all of the foregoing disadvantages are avoided. More particularly, in accordance with this invention, a delay-initiation cord characterized by uniform low velocity, low brisance and the production of little noise is provided which comprises a continuous core of a deflagrating composition encased in snug peripheral engagement by a flexible sheath having a tensile strength of at least about 25 p.s.i., the loading of the deflagrating composition in the core being from 0.1 to 5 grains per foot, the said core of deflagrating composition being characterized by a uniform deflagration velocity of from 100 to 650 meters per second.

More specifically, the delay-initiation cord of this invention comprises a core of deflagrating composition encased in snug peripheral engagement by a sheath of flexible material having a tensile strength of at least 25 p.s.i., said composition being selected from the group consisting of (A) a composition containing from 75 to 98 parts by weight lead azide and from 25 to 2 parts by weight non-explosive diluent, said core having a packed density of at least 3.5 g./cc.; (B) a composition selected from the group consisting of (1) tetracene and (2) mixtures of the lead salt of dinitro-o-cresol with a member of the group consisting of (a) potassium chlorate and tetracene, (b) potassium chlorate and pentaerythritol tetrinitrate, (c) potassium chlorate and lead styphnate, and (d) potassium chlorate and diazodinitrophenol; and (C) a composition containing from about 10 to about 90 parts by weight lead azide and from about 90 to about 10 parts by weight of an explosive composition selected from the group consisting of nitromannite, pentaerythritol tetrinitrate, tetracene, and diazodinitrophenol; said core of deflagrating composition being at a packed density of at least 3.5 g./cc. and being characterized by a uniform deflagration velocity of from 100 to 650 meters per second.

While the deflagration velocity for the deflagrating composition is given as 100 to 650 meters per second, this is equivalent to a burning rate of from about 3.0 to 0.5 millisecond per foot.

By the term "deflagration composition" is meant that the composition, when properly initiated, propagates a

"deflagration stimulus," i.e., a stimulus produced by a chemical reaction characterized by the vigorous evolution of heat and sparks or flame and moving through the material deflagrating at a speed less than that of sound, generally at a speed less than about 2000 meters per second.

The term "packed density" as used herein denotes the density of the core after the necessary steps in the processing of the cord have been completed.

In a preferred embodiment of this invention, the core of deflagrating composition is at a loading of about 0.1 to 2 grains per foot and the composition comprises about 75 to about 98 parts by weight of lead azide and 25 to about 2 parts by weight of a diluent such as a non-explosive composition; e.g., graphite, calcium stearate, methyl cellulose, polychlorinated polyphenols, modified fatty esters, polyisobutylene, dextrin, wax, talc, neoprene, lead carbonate, red lead, ammonium phosphate, polyvinyl acetate, and chlorosulfonated polyethylene. The packed density of the core must be at least 3.5 g./cc. and preferably from about 3.7 to about 4.5 g./cc. To insure that the stimulus transmitted by the cord is of deflagrating nature, initiation of the core should be by a low-energy shock such as is provided when the cord is actuated through its sheath by detonating fuse, i.e., by wrapping it around "Primacord," or "side-printed" by an initiator, i.e., the initiator is taped side-by-side to the cord rather than end-to-end in the conventional manner. However, cords whose cores have a packed density of greater than about 4.3 g./cc. can be initiated at the desired low velocities by initiators taped end-to-end.

In another preferred embodiment of this invention, the core is of a normally deflagrating composition such as tetracene; a mixture of the lead salt of dinitro-o-cresol, potassium chlorate and PETN; a mixture of the lead salt of dinitro-o-cresol, potassium chlorate and lead styphnate, or a mixture of the lead salt of dinitro-o-cresol, potassium chlorate, and diazodinitrophenol. These cords are reliably initiated at low, deflagrating velocities either when attached to an electric or non-electric initiator in the conventional manner (end-to-end) or when knotted or coiled about or taped to detonating fuse.

In still another preferred embodiment of this invention, the deflagrating core comprises from about 10 to about 90 parts by weight of lead azide, the balance of the core composition being a normally explosive composition such as PETN, nitromannite, tetracene, or diazodinitrophenol, and the loading of the core is preferably from about 0.1 to about 1.5 gr./ft. In this case, as in the case of the lead azide/diluent cores, the density of the core should be high, e.g., above 3.5 g./cc., as provided when the cord is prepared by swaging, and initiation should be through the sheath, either by wrapping the cord around "Primacord" and initiating the "Primacord" or by side priming with a conventional explosive initiator.

The delay-initiation cord of this invention can be used as the delay means in a delay blasting assembly comprising a plurality of boreholes loaded with high explosive charges, a downline of detonating fuse extending from the ground surface to the desired depth within the borehole (usually the full length of the boreholes), a plurality of lengths of delay-initiation cord connecting said downlines in a predetermined sequential relationship and a means for initiating the assembly, at least one end of said lengths of delay-initiation cord being capped by a metal shell containing an explosive charge initiatable by the deflagration impulse of said cord and of sufficient strength to initiate detonating fuse.

Alternatively, the delay-initiation cord of this invention can be used in a delay blasting assembly as the downline extending into the borehole with the downlines connected in the predetermined sequential relationship by detonating fuse. The length of the downline in each borehole is directly proportional to the delay time de-

sired between initiation of the assembly and actuation of the charges in the borehole. In this assembly, one end of the delay-initiation cord is attached to the detonating fuse, which initiates the downline, and the other end is capped by a shell containing an explosive train initiatable by the deflagration impulse from said cord and producing an impulse of sufficient strength to actuate an initiator for the charges in the borehole.

The accompanying figures illustrate various practical embodiments of this invention. In the drawings,

FIGURE 1 is a schematic top view of a quarry face and shows a typical blast layout in accordance with my invention,

FIGURES 2, 3, and 4 show various alternative means of connecting my delay-initiation cord to detonating fuse,

FIGURE 5 is a schematic representation in cross section of the delay-initiation cord,

FIGURE 6 is a sectional view of a borehole showing a typical blast layout in accordance with my invention.

Referring now to FIGURE 1 for more detailed explanation of the assembly of my invention, the edge of the quarry face is indicated at F. Boreholes indicated by B are drilled vertically in the face in three rows, each row having seven holes spaced apart a distance of 20 feet. Each borehole, which is loaded with explosive charges and has inserted its full depth a downline of detonating fuse as the primer, is connected to the adjacent boreholes by a length of delay-initiation cord A and each row of holes is connected to the one originally initiated. In this case, a second parallel length of the same cord, A', has also been employed to provide maximum assurance against failures or cutoffs. Cords A and A' are initiated at point I by initiator E, which in this case is an electric initiator. Assuming that cords A and A' have a burning rate of 1 millisecond per foot and are 20 feet long, the charges in holes B<sub>2</sub> and B<sub>1</sub>' are initiated after a time delay of 20 milliseconds after initiation of the charges in the initial borehole B<sub>1</sub>, the charges in holes B<sub>1</sub>', B<sub>2</sub>', and B<sub>3</sub> after 40 milliseconds, and so on until all the holes have been shot. Obviously, if a longer delay interval, e.g., 22 or 25 milliseconds, if desired, the length of the delay-initiation cord will be chosen accordingly.

In FIGURE 2, P indicates a length of detonating fuse provided as the primer or down-line for the explosive charges in a borehole. Delay-initiation cord A is connected to fuse P through initiator G which is securely attached side-by-side to the fuse by tape T. A second length of cord A is knotted around fuse P at a point below the initiator G and extends to the next borehole. Initiator G on actuation by cord A initiates fuse P, which in turn initiates the second length of cord A knotted around it. Cord A then relays the delay initiation stimulus to the corresponding initiator G in the adjacent borehole.

In the assembly of FIGURE 3, devised to relay the initiation stimulus in either direction, P, G, T, and A are as in the assembly of FIGURE 2 except that the initiators are attached perpendicularly to fuse P rather than side-by-side. In this case, if the delayed initiation stimulus comes through cord A, initiator G' will initiate fuse P and cord A' will carry the delayed initiation stimulus to the adjacent borehole. On the other hand, if the initiation stimulus comes from the direction of cord A', initiator G will initiate fuse P and the delayed initiation impulse will be directed along cord A. For convenience, the initiators may be contained in a plastic or metal shell having a transverse hole to receive detonating fuse.

FIGURE 4 shows a modification of the two-way assembly of FIGURE 3 wherein the initiators G and G' are positioned side-by-side and parallel to the fuse P rather than perpendicular thereto.

In the delay-initiation cord illustrated by FIGURE 5,

M is a continuous core of a deflagrating composition, N is a sheath of a ductile metal or a woven textile such as high denier rayon, and O represents a layer of water-proofing and strengthening material, e.g., a plastic and/or textile covering.

In FIGURE 6, B represents a vertical borehole containing conventional cap-sensitive explosive units U, the bottom-most charge being indicated at S. In intimate relationship with the bottom unit is initiator G which is attached to delay-initiation cord A. This delay-initiation cord A extends from the bottom of the borehole past explosive units U and through stemming T to the surface of the borehole where it is attached to detonating fuse P connecting this borehole with other boreholes in the blasting assembly. The delay-initiation cord may extend only from the bottom of the borehole to the top or it may extend from the bottom of the borehole to a point remote from the top of the borehole, or a long length of the cord can be coiled or looped so that a long length of the cord can be present in the borehole. In any event, the interval or delay between actuation of the cord by the detonation fuse and the time when the deflagration stimulus transmitted by the cord actuates initiator G in the borehole is directly proportional to the length of delay-initiation cord used. For example if the length of delay-initiation cord within the borehole is 20 feet and the burning rate of the cord is 1 millisecond per foot, the delay between the time when the cord is actuated by the detonating fuse and the time when the deflagration stimulus is transmitted to initiator G will be 20 milliseconds. If a different delay interval is desired, the length of the delay-initiation cord will be chosen accordingly. For example, a 20 millisecond interval may be desired between firing of this borehole and firing of the charges in the next borehole in the round in which case the length of delay-initiation cord in the next borehole would be 40 feet. Since the detonating fuse propagates the initiation impulse at a velocity of above 5000 meters per second, initiation of the two lengths can be considered essentially simultaneous, so that there will be a 20 millisecond interval (40 milliseconds minus 20 milliseconds) between actuation of the charges in the first borehole and actuation of charges in the second borehole.

The delay-initiation cords of this invention are prepared by filling the tubular sheath which preferably is of a ductile metal such as of lead or aluminum, with the desired deflagrating agent and subsequently drawing or swaging the sheath to reduce the diameter and to increase the density of the core. After the drawing or swaging step, the cord may be covered with a layer of water-proofing and reinforcing material such as a bituminous coating, spirally applied yarn, a wax finish, or a single extruded coating of a thermoplastic or thermosetting resin, preferably polyethylene or polyvinyl chloride. Alternatively, the tubular sheath may be woven of fibers such as of heavy denier (e.g., about 300 denier) rayon, cotton, or nylon.

For cords containing lead azide as a major constituent of the core composition, I have found that swaging of the tubular sheath gives a cord of more uniform deflagrating characteristics than does drawing since by this method, wherein the tube is struck by a large number of successive blows by a pair of shaped dies, higher core densities can be achieved. As further insurance of obtaining the high densities necessary particularly for core compositions containing lead azide, the fill density of the core should be at least about 2.4 g./cc. and preferably should be greater than 2.7 g./cc. since with this fill density, the density of the core can readily be increased to the 3.5 g./cc. required for reliable propagation of a deflagration stimulus. As noted above, to insure propagation of a deflagration stimulus with lead azide compositions it is also necessary that the composition contain from about 2 to about 25% of a diluent. Exemplary diluents include non-explosive compositions such

as graphite, calcium stearate, methyl cellulose, poly-chlorinated polyphenols, modified fatty esters, poly-isobutylene, dextrin, wax, talc, neoprene, lead carbonate, red lead, ammonium phosphate, polyvinyl acetate, chlorosulfonated polyethylene, and the like. Although cores containing higher percentages of lead azide can propagate a deflagration stimulus when at high densities, i.e., at densities greater than about 4.3 g./cc., when initiated by side priming or by wrapping around "Primacord," these compositions do not reliably propagate a deflagration stimulus at lower densities and, accordingly, may propagate either a deflagration or detonation stimulus. When more than about 25% of a nonexplosive diluent is present in the core compositions, the velocity at which an impulse is propagated becomes so slow as to be unreliable for precision blasting operations. Within the specified ranges however, the cords propagate a deflagration stimulus at a uniform, precise rate.

The following examples illustrate specific embodiments of the delay-initiation cord of this invention.

#### EXAMPLE 1

A series of lead-sheathed cords containing various lead azide/diluent compositions were prepared by loading lead tubes having an outside diameter of about 0.312 inch, and an inside diameter of about 0.157 inch, with these compositions at a filling density of approximately 2.4 g./cc. and reducing the diameters of the tubes by swaging. In each case, the lead azide used was commercially available dextrinated lead azide which has a lead azide content of 93%. The cords, their core compositions and loadings and their velocity of deflagration are summarized in the following table (Table 1), wherein "lead azide" denotes the above-described dextrinated lead azide. In each case, the cords were initiated by wrapping them around "Primacord" and initiating the "Primacord." In each case after the cords were swaged, the packed density of each core was at least 3.5 g./cc. and, generally, about 3.7 g./cc.

Table 1

|    | Core Composition                                       | Core Loading (gr./ft.) | Velocity, m./sec. |
|----|--------------------------------------------------------|------------------------|-------------------|
| 40 | 80/20 lead azide/barium peroxide.....                  | 1                      | 600               |
|    | Do.....                                                | 2                      | 660               |
| 45 | 97.5/2.5 lead azide/Bareco wax.....                    | 1                      | 330               |
|    | Do.....                                                | 2                      | 390               |
| 50 | 98/2 lead azide/Bareco wax.....                        | 1                      | 280               |
|    | 97/3 lead azide/Bareco wax.....                        | 1                      | 190               |
|    | 96/4 lead azide/Bareco wax.....                        | 1                      | 120               |
|    | 95/5 lead azide/Bareco wax.....                        | 1                      | 100               |
|    | 98/2 lead azide/Neoprene.....                          | 1                      | 490               |
|    | Do.....                                                | 2                      | 540               |
| 55 | 98.8/1.2 lead azide/methyl cellulose.....              | 1                      | 620               |
|    | 92/8 lead azide/polyvinyl acetate.....                 | 1                      | 480               |
|    | 98.5/1.5 lead azide/chlorosulfonated polyethylene..... | 1                      | 440               |
|    | Do.....                                                | 2                      | 450               |
| 60 | 95/5 lead azide/diabasic lead phosphate.....           | 1                      | 620               |
|    | 95/5 lead azide/lead carbonate.....                    | 1                      | 635               |
|    | Do.....                                                | 2                      | 575               |
|    | 90/10 lead azide/lead carbonate.....                   | 1                      | 600               |
|    | 85/15 lead azide/lead carbonate.....                   | 2                      | 580               |
|    | 80/20 lead azide/lead carbonate.....                   | 1                      | 355               |
|    | 90/10 lead azide/red lead.....                         | 1                      | 625               |
|    | 98.8/1.2 lead azide/polyisobutylene.....               | 1                      | 480               |
|    | 97/3 lead azide/conductive wax.....                    | 1                      | 490               |
| 65 | 97/3 lead azide/polychlorinated polyphenol.....        | 1                      | 270               |
|    | 99/1 lead azide/polychlorinated polyphenol.....        | 1                      | 455               |
|    | 90/10 lead azide/ammonium phosphate.....               | 1                      | 430               |
|    | 90/10 lead azide/talc.....                             | 1                      | 390               |
|    | 97/3 lead azide/fatty ester.....                       | 1                      | 230               |
|    | Do.....                                                | 2                      | 240               |
|    | 98/2 lead azide/Glycowax.....                          | 1                      | 240               |
|    | Do.....                                                | 2                      | 280               |
| 70 | 98/2 lead azide/wax.....                               | 1                      | 260               |
|    | 99.5/0.5 lead azide/wax.....                           | 1                      | 455               |

When cords were prepared using higher purity lead azide, i.e., colloidal lead azide (99% lead azide) and a composition having a lead azide content of 98% as the sole component of the core and initiated by "Primacord," predominately high detonating velocities (3900-4000 meters/second) were exhibited, even at core loadings of less than 1/2 gr./ft., in swaged lead tubes.

75 In order to evaluate the relationship of core density

and method of initiation to the deflagration velocity of the cord, a series of cords were prepared as in Example 1 by swaging. At the same time, a series of cords were prepared for comparative purposes using the same core loadings and compositions, however, in these cords prepared for comparative purposes, the reduction of lead tubes containing the lead azide/diluent was accomplished by drawing through dies so that the packed densities of the cores were less than the 3.5 g./cc. value, which I have found necessary to insure that a deflagration stimulus is transmitted by the cord. Initiation of the cords was effected (a) by butting the cord against a conventional blasting cap (end-to-end) and (b) by wrapping the cords about a length of "Primacord." The cords, their core compositions and loadings and their velocity of deflagration (or detonation) are summarized in the following table (Table 2). As in Table 1, the lead azide referred to is dextrinated lead azide having a lead azide content of 93%.

Table 2

| Composition                         | Preparation Method | Velocity, m./sec.    |                        |                      |                        |
|-------------------------------------|--------------------|----------------------|------------------------|----------------------|------------------------|
|                                     |                    | Loading of 1 gr./ft. |                        | Loading of 2 gr./ft. |                        |
|                                     |                    | Cap Initiation       | "Primacord" Initiation | Cap Initiation       | "Primacord" Initiation |
| 80/20 lead azide/barium peroxide    | Drawing            | 2,400                | 2,500                  | 2,600                | 2,900                  |
| Do                                  | Swaging            | 630                  | 600                    | 3,140                | 660                    |
| 97/2.5 lead azide/Bareco wax        | Drawing            | 2,600                | 2,720                  | 2,850                | 2,880                  |
| Do                                  | Swaging            | 310                  | 330                    | 2,960                | 320                    |
| 98/2 lead azide/Neoprene            | Drawing            | 2,650                | 2,820                  | 2,770                | 2,850                  |
| Do                                  | Swaging            | 3,400                | 490                    | 3,720                | 540                    |
| 92/8 lead azide/polyvinyl acetate   | Drawing            | 2,300                | 2,420                  | 2,440                | 2,650                  |
| Do                                  | Swaging            | 3,280                | 480                    | 3,430                | 470                    |
| 95/5 lead azide/lead carbonate      | Drawing            | 2,600                | 2,480                  | 2,580                | 2,580                  |
| Do                                  | Swaging            | 3,370                | 635                    | 3,390                | 575                    |
| 90/10 lead azide/lead carbonate     | Drawing            | 2,600                | 2,200                  | 2,820                | 2,460                  |
| Do                                  | Swaging            | 3,250                | 660                    | 3,175                | 570                    |
| 98.8/1.2 lead azide/polyisobutylene | Drawing            | 2,540                | 2,700                  | 2,880                | 2,900                  |
| Do                                  | Swaging            | 3,315                | 480                    | 3,315                | 510                    |
| 97/3 lead azide/conductive wax      | Drawing            | 2,680                | 2,750                  | 2,880                | 2,820                  |
| Do                                  | Swaging            | 3,430                | 490                    | 3,470                | 470                    |

Cord "side-primed" by conventional electric blasting cap demonstrated essentially the same velocities as cord initiated by "Primacord."

As may be seen from the table, when lead azide compositions are used as the deflagrating core in the delay-initiation cord of this invention, (a) a diluent must be present, (b) the density of the cord must be at least 3.5 g./cc., i.e., the cord should be prepared by swaging, or pressurized by other means such as hydrostatic pressure, and (c) initiation of the cord should be by a low-energy shock such as is provided when the cord is wrapped around "Primacord" or when side-primed by an initiator.

## EXAMPLE 2

A series of delay-initiation cords were prepared by the swaging technique described in Example 1, using dextrinated lead azide (93% lead azide) as the core composition. Various lengths of the cord were cut and initiated by wrapping them around "Primacord." Results of timing tests are shown below.

Table 3

| Loading, gr./ft. | Length of Cord, ft. | Time, ms. | Velocity, m./sec. | Burning rate, ms./ft. |
|------------------|---------------------|-----------|-------------------|-----------------------|
| 0.78             | 1 1/2               | 1.44      | 312               | 0.96                  |
| 0.78             | 2                   | 1.84      | 332               | 0.92                  |
| 0.78             | 3 1/2               | 3.13      | 341               | 0.89                  |
| 0.78             | 10                  | 9.15      | 333               | 0.92                  |
| 0.78             | 10                  | 9.26      | 329               | 0.93                  |
| 1                | 2                   | 1.25      | 487               | 0.63                  |
| 1                | 2                   | 1.26      | 485               | 0.63                  |
| 1                | 5                   | 3.12      | 489               | 0.62                  |
| 1                | 5                   | 3.12      | 488               | 0.63                  |
| 1                | 10                  | 6.27      | 487               | 0.63                  |
| 1                | 10                  | 6.29      | 485               | 0.63                  |
| 1                | 20                  | 12.51     | 487               | 0.63                  |
| 1                | 20                  | 12.36     | 493               | 0.62                  |

were prepared in swaged 0.073 inch diameter lead tubes (core load of 1.4 gr./ft.; packed density above 3.5 g./cc.).

## Lead azide/nitromannite

90/10  
80/20  
50/50  
40/60  
25/75  
20/80  
10/90

In general velocities of the cords were in the range of 500-550 m./sec. when the cords were initiated by "Primacord." Typical, average velocity measurements for 75/25 nitromannite/lead azide swaged in 0.073 diameter lead sheaths (core loading of 1.4 gr./ft.) were about 492 m./sec.

60 Similar results were obtained for lead azide/fine PETN cores as shown below at loadings of 0.5 and 1 gr./ft. were tested in swaged lead sheaths.

## Lead azide/PETN

90/10  
50/50  
25/75  
10/90

Tests on 80/20, 90/10, 95/5, and 98/2 lead azide/tetraene mixtures indicated that material in drawn lead tubings transmitted a deflagration stimulus when initiated by "Primacord" and that material swaged in lead at core loadings of less than 1 gr./ft. burned at low deflagration

velocities both for "Primacord" and end-to-end cap initiation. Results for 90/10 lead azide/tetracene compositions are shown in Table 4.

Table 4

| Loading, gr./ft. | Outside diameter, inches | Velocity, m./sec. | Burning rate, ms./ft. |
|------------------|--------------------------|-------------------|-----------------------|
| 2.43             | 0.15                     | 410               | 0.743                 |
| 1.10             | 0.105                    | 368               | 0.829                 |
| 0.58             | 0.073                    | 335               | 0.910                 |

## EXAMPLE 5

Delay-initiation cords were prepared by the swaging procedure described in Example 1, except that tetracene alone was used as the core composition. The cords functioned as shown in Table 5, below.

Table 5

| Loading, gr./ft. | Outside diameter, inches | Initiator   | Burning rate, ms./ft. | Velocity, m./sec. |
|------------------|--------------------------|-------------|-----------------------|-------------------|
| 3.08             | 0.150                    | Cap         | 1.142                 | 267               |
| 3.08             | 0.150                    | "Primacord" | 1.128                 | 270               |
| 1.46             | 0.105                    | Cap         | 1.134                 | 269               |
| 1.46             | 0.105                    | "Primacord" | 1.174                 | 260               |
| 0.073            | 0.073                    | Cap         | 1.172                 | 260               |
| 0.073            | 0.073                    | "Primacord" | 1.032                 | 295               |
| 0.36             | 0.051                    | Cap         | 0.949                 | 321               |
| 0.36             | 0.051                    | "Primacord" | 0.865                 | 352               |

| 5  | Composition                   |                    | Loading (gr./ft.) | Velocity, m./sec. | Burning Rate, ms./ft. |
|----|-------------------------------|--------------------|-------------------|-------------------|-----------------------|
|    | Lead salt of dinitro-o-cresol | Potassium chlorate |                   |                   |                       |
| 10 | 80                            | 20                 | 1.2               | 200               | 1.52                  |
|    | 80                            | 20                 | 0.6               | 203               | 1.50                  |
|    | 80                            | 20                 | 0.3               | 170               | 1.79                  |
|    | 70                            | 30                 | 1.3               | 236               | 1.29                  |
|    | 70                            | 30                 | 0.64              | 238               | 1.28                  |
|    | 70                            | 30                 | 0.34              | 233               | 1.31                  |
|    | 70                            | 30                 | 0.21              | 210               | 1.45                  |
|    | 70                            | 30                 | 0.16              | 201               | 1.52                  |
|    | 70                            | 30                 | 0.08              | 180               | 1.69                  |
|    | 60                            | 40                 | 2.6               | 235               | 1.30                  |
| 15 | 60                            | 40                 | 1.4               | 241               | 1.27                  |
|    | 60                            | 40                 | 0.73              | 231               | 1.32                  |
|    | 50                            | 50                 | 6.6               | 212               | 1.44                  |
|    | 50                            | 50                 | 3.3               | 229               | 1.33                  |
|    | 50                            | 50                 | 1.9               | 220               | 1.39                  |
|    | 50                            | 50                 | 0.97              | 228               | 1.34                  |
|    | 50                            | 50                 | 0.55              | 239               | 1.28                  |
|    | 40                            | 60                 | 5.6               | 217               | 1.40                  |
|    | 40                            | 60                 | 2.7               | 216               | 1.41                  |
|    | 40                            | 60                 | 1.4               | 212               | 1.44                  |
| 20 | 40                            | 60                 | 0.67              | 209               | 1.46                  |
|    | 40                            | 60                 | 0.49              | 210               | 1.45                  |

25

## EXAMPLE 7

A series of cords containing various mixtures of the lead salt of dinitro-o-cresol, potassium chloride, and tetracene were prepared by the drawing and swaging methods of Examples 1 and 6. The composition and loading of the cores, the method used in their preparation, the deflagration velocities and the burning rates of the cords are summarized in Table 7.

35

Table 7

| Lead Salt of 1,2-dinitro-o-cresol | Composition        |            |      | Loading, gr./ft. | Preparation Method | Velocity, m./sec. | Burning Rate, ms./ft. |
|-----------------------------------|--------------------|------------|------|------------------|--------------------|-------------------|-----------------------|
|                                   | Potassium Chlorate | Tetra-cene |      |                  |                    |                   |                       |
| 50                                | 40                 | 10         | 2    | Drawing          | 290                | 1.05              |                       |
| 50                                | 40                 | 10         | 1    | do               | 277                | 1.10              |                       |
| 50                                | 40                 | 10         | 3    | do               | 283                | 1.11              |                       |
| 50                                | 35                 | 15         | 3.35 | do               | 287                | 1.06              |                       |
| 50                                | 35                 | 15         | 0.94 | do               | 292                | 1.04              |                       |
| 50                                | 45                 | 5          | 3.05 | do               | 298                | 1.02              |                       |
| 50                                | 45                 | 5          | 2.19 | do               | 279                | 1.09              |                       |
| 50                                | 45                 | 5          | 1.56 | do               | 263                | 1.16              |                       |
| 50                                | 45                 | 5          | 1.07 | do               | 265                | 1.15              |                       |
| 50                                | 45                 | 5          | 0.05 | do               | 251                | 1.21              |                       |
| 50                                | 40                 | 10         | 2.85 | do               | 225                | 1.36              |                       |
| 50                                | 40                 | 10         | 1.95 | do               | 210                | 1.46              |                       |
| 50                                | 40                 | 10         | 0.95 | do               | 197                | 1.55              |                       |
| 50                                | 40                 | 10         | 0.93 | Swaging          | 241                | 1.26              |                       |
| 50                                | 40                 | 10         | 0.54 | do               | 242                | 1.26              |                       |
| 50                                | 40                 | 10         | 0.50 | do               | 248                | 1.23              |                       |

## EXAMPLE 6

A series of cords were prepared by loading mixtures of the lead salt of dinitro-o-cresol and potassium chloride at different percentage compositions into lead tubes, closing the tube, e.g., with cotton, and drawing the tubes through successively smaller dies down to the desired core loadings and tube diameters. The core compositions, in parts by weight, loadings, deflagration velocities, and burning rates of the cords are summarized in Table 6. In each case, the cords were initiated by a conventional blasting cap butted against a cut end of the cord (end-to-end initiation).

65 A delay-initiation cord was prepared using 50/40/10 mixtures of the lead salt of dinitro-o-cresol/potassium chloride/fine PETN at a loading of 0.56 gr./ft. in a drawn lead tube. When the cord was initiated by a conventional electric blasting cap (end-to-end initiation) the cord propagated a deflagration stimulus at a velocity of 70 225 m./sec. (1.34 m./ft.).

75 EXAMPLE 9  
Delay-initiation cords were prepared by the drawing technique with 1 and 2.3 gr./ft. core loadings of 50/40/10 lead salt of dinitro-o-cresol/potassium chlorate/lead styph-

## EXAMPLE 8

nate and were initiated by end-to-end priming with an electric blasting cap. The cords burned at deflagration velocities of 240-250 m./sec.

#### EXAMPLE 10

The deflagration velocity of a cord containing a 50/40/10 lead salt of dinitro-o-cresol/potassium chlorate/diazodinitrophenol composition at a loading of 1.17 gr./ft. in drawn lead tubing was 227 m./sec. when initiated by end-to-end priming by an electric blasting cap. The velocities of swaged cords having core loads 1.67 and 0.83 gr./ft. of the composition varied from about 231-246 m./sec.

The delay-initiation cord of this invention is characterized by uniform low velocity, low brisance, and the production of little noise. Therefore, the cord is particularly advantageous for use in applications where shielding cannot be provided, for example in "bottom-hole priming" where the noise and brisance inherent in detonating fuse and delay connectors cannot be tolerated. The low brisance of the cord eliminates the possibility of simultaneous deflagration of all the cord composition within a coiled length, and the deflagration generally is propagated through the core without damaging the counteracting at all. Since the cord is flexible, the blasting operator may choose the length of delay-initiation cord appropriate to the amount of time delay desired and, if necessary, coil or bend the cord to fit the spatial confines of his blasting assembly. This continuity of propagation even through a knotted or kinked section is surprising in view of the known failure of ignition-transmission lines which depend upon the oversize conduit for burning combustible materials to propagate through knots or kinks.

It will be apparent from the foregoing that the delay-initiation cord of this invention fills a void in the art in that it provides a highly efficient and dependable flexible delay-initiation cord which makes possible the elimination of the costly and undependable delay devices heretofore considered necessary and provides highly efficient and dependable delay action at a cost appreciably below those in present-day conventional practice.

The present invention has been described in detail in the foregoing. However, as will be apparent to those skilled in the art, variations are possible without departure from the scope of the invention.

What is claimed is:

1. A delay-initiation cord comprising a core of deflagrating composition containing from 75 to 98 parts by weight lead azide and from 25 to 2 parts by weight non-explosive diluent, encased in a sheath of a flexible material having a tensile strength of at least 25 pounds per square inch, the loading and the packed density of said deflagrating composition being from about 0.1 to 2 grains per foot and at least 3.5 g./cc. respectively, and said core of deflagrating composition being characterized by a uniform deflagration velocity of from 100 to 650 meters per second.

2. The cord as in claim 1 wherein said non-explosive

diluent is selected from the group consisting of graphite, calcium stearate, methyl cellulose, polychlorinated polyphenols, modified fatty esters, polyisobutylene, dextrin, wax, talc, neoprene, lead carbonate, red lead, ammonium phosphate, polyvinyl acetate, and chlorosulfonated polyethylene.

3. The cord of claim 1 wherein said sheath is of ductile metal and the core of deflagrating composition is at a packed density of about from 3.7 to 4.5 g./cc.

4. A delay-initiation cord comprising a core of deflagrating composition selected from the group consisting of (1) tetracene and (2) mixtures of the lead salt of dinitro-o-cresol with a member of the group consisting of (a) potassium chlorate and tetracene, (b) potassium chlorate and pentaerythritol tetranitrate, (c) potassium chlorate and lead styphnate, and (d) potassium chlorate and diazodinitrophenol, encased in a sheath of a flexible material having a tensile strength of at least 25 pounds per square inch, the loading of said deflagrating composition being from about 0.1 to 5 grains per foot, and said core of deflagrating composition being characterized by a uniform deflagration velocity of from 100 to 650 meters per second.

5. The cord of claim 4 wherein said sheath is of ductile metal.

6. A delay initiation cord comprising a core of deflagrating composition containing from about 10 to about 90 parts by weight lead azide and from about 90 to about 10 parts by weight of an explosive composition selected from the group consisting of nitromannite, pentaerythritol tetranitrate, tetracene, and diazodinitrophenol, encased in a sheath of a flexible material having a tensile strength of at least 25 pounds per square inch, the loading and the packed density of said deflagrating composition being from about 0.1 to 1.5 grains per foot and at least 3.5 g./cc. respectively, and said core of deflagrating composition being characterized by a uniform deflagration velocity of from 100 to 650 meters per second.

7. The chord of claim 6 wherein said sheath is of ductile metal.

#### References Cited by the Examiner

##### UNITED STATES PATENTS

|           |       |                      |        |
|-----------|-------|----------------------|--------|
| 2,175,249 | 10/39 | Burrows et al. ----- | 149-24 |
| 2,239,123 | 4/41  | Stoneking -----      | 102-23 |
| 2,865,726 | 12/58 | Jenkins et al. ----- | 149-35 |
| 2,923,239 | 2/60  | Andrew et al. -----  | 102-27 |
| 2,980,019 | 4/61  | Noddin -----         | 102-28 |
| 2,982,210 | 5/61  | Andrew et al. -----  | 102-27 |
| 2,992,611 | 7/61  | Felch -----          | 102-22 |

##### FOREIGN PATENTS

731,108 6/55 Great Britain.

SAMUEL FEINBERG, Primary Examiner.